

Aug. 3, 1948.

H. STEWART ET AL

2,446,514

SEPARATION OF HYDROCARBON MIXTURES

Filed Sept. 16, 1944



Inventors: Hall Stewart  
August A. Schaefer

By their Attorney: 8 Cusack

## UNITED STATES PATENT OFFICE

2,446,514

## SEPARATION OF HYDROCARBON MIXTURES

Hall Stewart, Oakland, and August A. Schaefer, El Cerrito, Calif., assignors to Shell Development Company, San Francisco, Calif., a corporation of Delaware

Application September 16, 1944, Serial No. 554,486

14 Claims. (Cl. 196—14.48)

1

This invention involves a process for separating oils of different degrees of aromaticity and paraffinicinity from a liquid hydrocarbon mixture. More particularly, it deals with a process for producing a high viscosity index oil from lubricating oils.

The process is based upon the discovery that when lubricating oil containing solid wax and high and low viscosity index oil components in a solution of a solvent for aromatic hydrocarbons is gradually chilled, it will become thicker and thicker, forming a gelatinous slurry until all at once a temperature is reached where a granular solid precipitate is produced of substantially all the non-aromatic hydrocarbons.

It is a purpose of this invention to simply, economically, and effectively separate liquid non-aromatic hydrocarbons from liquid aromatic hydrocarbons in a mixture thereof heavier than kerosene. Another purpose is to produce high viscosity index oils from lubricating oil of lower viscosity index. Another purpose is to produce a highly refined high viscosity index oil in a simple and effective manner. Another purpose is to simply, economically and efficiently separate crystalline and amorphous waxes (petrolatum) from each other. Other purposes are to fractionate solid waxes, separate straight chain type paraffins from naphthenes and branched chain type hydrocarbons, etc.

Generally speaking this invention comprises mixing a hydrocarbon oil having an average molecular weight above that of kerosene, comprising aromatic and non-aromatic hydrocarbons and containing between about 5% and 25% normally solid wax with a solvent selective for aromatic hydrocarbons, chilling the resulting mixture to solidify relatively non-aromatic hydrocarbons (paraffinic and/or naphthenic oil and wax) as a filterable precipitate, and filtering this precipitate from the resulting liquid solvent containing dissolved aromatic hydrocarbons. The separated precipitate is then refractionated by a similar operation at a higher temperature to separate solidified wax. If desired, the solid waxes may be separated into amorphous and crystalline waxes by a similar treatment at still higher temperatures. The solvent in the filtrates of each step may be removed from the oils by any suitable means, such as distillation, and re-used in the process.

The terms "aromatics" vs. "non-aromatics" and "paraffins and/or naphthenes" vs. "aromatics" as used herein are all relative to each other, de-

2

pending upon the composition of the oil being treated.

The presence of normally solid paraffin wax in the oil-solvent mixture is necessary to enable precipitation of the major portion of the non-aromatic hydrocarbons in an easily filterable form, thereby making possible an easy and effective washing of the filter cake. When chilling a lubricating oil in solution of selective solvent to a very low temperature and a portion of the oil begins to precipitate, the mixture becomes thick and jelly-like. As the temperature is further reduced, this condition becomes more aggravated. However, if solid wax is present, a sudden break occurs at a certain temperature: the gelatinous slurry suddenly becoming readily filterable. This break does not occur if solid wax is substantially absent. If the gelatinous slurry fails to break, the mixture filters only with difficulty and the cake retains large amounts of aromatic oil. It follows that, for a given yield of dewaxed paraffinic oil, a higher viscosity index is realized when carrying out the separation in the presence of paraffin wax rather than in its absence. In other words, the sequence of the separation should be: first separating aromatics from non-aromatics in the presence of wax and then dewaxing the non-aromatics to produce the high viscosity index dewaxed oil.

30 The break of the gelatinous slurry causes a sudden drop in the viscosity of the mixture as a result of which it becomes quite fluid. The temperature at which this break occurs and the precipitate becomes readily filterable is as a rule about  $-50^{\circ}$  C. or below, although it varies somewhat with different oils and solvents. For example, for most lubricating oil distillates using methyl ethyl ketone as the solvent, this temperature is between about  $-50^{\circ}$  and  $-60^{\circ}$  C. The break is probably due to a change in the crystalline forms of iso and cyclic paraffins in the mixture, and as indicated results in an abrupt reduction of the viscosity.

45 Washing of the filter cake is an important step where good separation is desired. It is because of this that filtration is superior to centrifuging as a separating method, because the wax separated by centrifuging cannot be washed as readily and economically.

50 Hydrocarbon oils which may be treated by the process of this invention should have an initial boiling temperature above about  $200^{\circ}$  C., and major portions should consist of components having at least 12 and preferably 15 or more carbon atoms per molecule. As indicated the oils

must contain dissolved at least 5% and not over 25%, preferably between 10% and 20%, of a normally solid wax, i. e. one which is solid at room temperature (20° C.). Since the wax acts only as a nucleus upon which the non-aromatic hydrocarbon oil may crystallize it is immaterial from what source it is derived. It may even be a natural wax ester such as a vegetable wax or an animal wax, provided it has a crystalline structure (micro-crystalline or otherwise). If the oil is deficient in wax, wax must be added. If it contains too much wax, it should be partially dewaxed to within the above limit, because such a large amount of wax serves no useful purpose in the oil and needlessly increases the volume of the filter cake and the cooling requirements. The oil must be substantially free from asphalts which stay in the oil when chilled because they inhibit the formation of filterable crystals by forming a gel. Hard asphalts, however, which remain in the wax when chilled may be tolerated or even may be added as a filter aid although they contaminate the wax. Nevertheless, it is desirable that the oil be deasphaltized prior to its separation by chilling by this process.

Suitable hydrocarbon oils may be derived from any crude containing aromatic and non-aromatic hydrocarbons, that is high and low viscosity index components. Distillate oils are easier to treat by this method than residual oils. In fact the latter may be very difficult to handle unless special means are employed. The narrower the fraction treated the closer the separation. Although wide lubricating oil fractions also may be treated with success, separation can be made between compositions having substantially the same or identical boiling temperatures. Pure crystalline waxes that contain compounds differing in not more than two carbon atoms per molecule may be produced by this process.

The solvent must be a polar solvent more selective for aromatic than for paraffinic hydrocarbons, that is, must have a greater solvency for aromatics than for paraffins. It must be stable and liquid at the temperatures employed in the process and must not become too viscous when chilled to temperatures near its freezing point. Preferably, the solvent is an organic solvent, since it must be completely miscible at room temperature with the hydrocarbon oils treated. It should be easily separated from the oils, say by distillation, that is, have a boiling temperature at least 10° C. outside the boiling range of the oils. It may consist of and/or comprise several liquids. The more selective the solvent for aromatic hydrocarbons the lower its solvent power for the wax and high viscosity index oil components. This results in the formation of a filterable precipitate of the non-aromatic and wax at a higher temperature, the formation of harder wax crystals, and easier filterability.

Some examples of suitable solvents are chlorinated hydrocarbons such as methyl chloride, ethylene dichloride, chloroform, etc.; alcohols such as isopropyl alcohol, secondary butyl alcohol, etc.; ketones such as acetone, methyl ethyl ketone, methyl n- and iso-propyl ketone, diisopropyl ketone, methyl isobutyl ketone, etc.; esters such as methyl and ethyl formates, acetates, propionates, etc. Ketones of 4-7 carbon atoms are preferred. The outstanding solvents are methyl ethyl ketone, methyl isopropyl ketone and methyl isobutyl ketone. Methyl ethyl ketone is the most selective but at extremely low temperatures may fall short of solvent power. The addition of a

minor proportion of benzene, toluene, xylenes, etc. will raise its solvent power. Methyl isobutyl ketone on the other hand has plenty of solvent power even at the lowest practical temperatures but is somewhat less selective. Therefore, methyl isobutyl ketone is often used in admixture with acetone or methyl ethyl ketone to increase its selectivity. Methyl isopropyl ketone stands between methyl ethyl ketone and methyl isobutyl ketone.

It is desirable to wash the filter cake with a polar solvent of the type just described, and preferably with the same solvent that is used in forming the precipitate. Fresh solvent may be used for the washing, and the wash liquor may then be used to effect the precipitation, after which the solvent may be recovered and recycled. The same or different solvents may be used in each separation and chilling operation, as desired.

The accompanying drawing shows a simplified flow diagram of one embodiment of this invention. Its description is divided into the following sections: (1) Separation of low viscosity index components, (2) Separation of high viscosity index components and (3) Separation of amorphous and crystalline waxes.

*I. Separation of low viscosity index components*

Referring to the drawing, the oil to be treated, which contains dissolved a solid wax content between about 5% and 25% by volume and both high and low viscosity index components, is fed through line 1 and admixed with solvent from line 2 in mixer 3. The resulting mixture is passed through line 4 to chillers 5 wherein it is agitated and chilled to a temperature sufficient to cause the "break" in the viscosity of the mixture, i. e. a temperature of -50° C. or below. The chilled solution then passes through line 6 to the filter 10 which, for convenience, has been shown as a vacuum rotating drum filter containing compartments so that the precipitate is sucked onto the porous drum surface 11 from the trough 12 and the filtrate (or liquid phase containing the solvent and low viscosity index components) is removed through line 13. The filter cake of precipitate comprising the waxes and the high viscosity index components rotates with the drum in the direction of the arrow and is washed with fresh or regenerated solvent pre-chilled in cooler 15 to the temperature of said cake by spraying it on the cake through lines 14. The spent wash solvent may be separately drawn from the center of the drum through line 16, or joined with the filtrate in line 13 either by elimination of the partition 17 in the drum or through valved line 18. Preferably, the spent wash solvent is passed through line 19 to line 2 and is used for admixing with the feed oil in line 1.

The filtrate and possibly the spent wash solvent, each of which contains some low viscosity index oil components, may be treated to remove the solvent, such as by distillation, in still 20 from which fresh solvent may be returned to line 14 through line 21, or to line 2 or other parts of the system (through lines not shown). The low viscosity index components are withdrawn as low viscosity index oil products through line 22. Fresh solvent may be introduced into this first separation step through line 7 joining line 2, or through line 23 joining line 14 as desired. The washed wax cake on drum 11 is scraped off and passed through line 24 to the next step in the

process for the removal of the high viscosity index components therein.

It is often desirable to remix with fresh solvent and refilter the wax precipitate two or even more times at this same temperature in order to obtain good separation. If this is done, less solvent is required to wash the precipitated wax cake and a higher viscosity index oil is obtained.

### II. Separation of high viscosity index components

The cold wax cake from line 24 is admixed with more solvent introduced through line 31 into mixer 30. The resulting mixture is then passed through line 32 into heat exchangers 33 wherein it is continuously agitated and heated (or cooled, as required) to a temperature above that employed in chillers 8, and dependent upon the pour point of the high viscosity index oil to be produced. The higher this temperature, the higher the pour point of the high viscosity index oil due to the presence of dissolved waxes; while the lower this temperature, the lower the pour point (and the viscosity index) of the high viscosity index oil due to the absence of dissolved waxes. For economy, the solvent and/or oil introduced in the first separation step I may be pre-cooled by heat exchange in exchangers 33. The resulting mixture, which contains a liquid phase of solvent and high viscosity index oil components and a solid phase of precipitated solid waxes, is then separated on a filter 34 and washed similarly to that described above in step I. Also, the solvent may be similarly recovered in still 35 and separated from the high viscosity index oil components which are withdrawn through line 36. The solid waxes may be removed through valved line 37 as product, recycled to blend with oil feed to make its wax content within the above limits, or further separated as described in the next step. The high viscosity index oils produced are highly refined and usually white. They are unstable to oxidation, but have good inhibitor susceptibilities.

Alternatively, this step II may comprise merely further washing the precipitated wax formed in step I with a warmer solvent than that used in the first step to dissolve the high viscosity index oil components from the normally solid waxes. However, this alternative method does not give as complete a separation as that described above.

### III. Separation of amorphous and crystalline waxes

The solid waxes from filter 34 are admixed with more solvent introduced through line 41 into mixer 40. The resulting mixture is continuously agitated in heat exchangers 43 until a temperature is reached which is higher than that in step II and which depends upon the melting point of the waxes desired. The higher melting or crystalline waxes are precipitated and the lower melting or amorphous waxes are dissolved in the solvent. The suspended solids are separated by such as filtering and washing on filter 44 and the crystalline wax is scraped off as a final product at 47. The amorphous wax is separated from the solvent in still 45 and withdrawn through line 46, while the recovered solvent may be recycled.

The described apparatus is merely illustrative of what may be employed in this process. For example, the chillers and heat exchangers may be of the Carbondale type and the filters may be of the Oliver, leaf, or other type, or they may be replaced by centrifuges or other suitable

means to separate suspended solids from a liquid.

Many of the necessary pipes, valves, tanks, pumps, heat exchangers, and the like are not shown in the drawing but their proper placement is within the knowledge of anyone skilled in the art.

The temperatures and solvent-to-feed ratios employed in each step of the process may vary with the type of solvent employed and the properties of the products to be produced. However, the temperature of the separation in step I is the lowest reached in the process, while the temperature in each succeeding step is progressively higher. The more selective the solvent is for aromatics and low viscosity index components, the higher may be the temperature in order to obtain the filterable precipitate required in step I. If low viscosity index oil, high viscosity index oil, amorphous waxes and crystalline waxes are the products, the temperature for step I is below about  $-50^{\circ}$  C.; for step II is between about  $-30^{\circ}$  C. and  $0^{\circ}$  C.; and for step III is between about  $0^{\circ}$  C. and  $20^{\circ}$  C.

The solvent-to-oil ratios vary with the type of solvent. For example in step I, the ratio ranges from about 1:1 to 10:1, and preferably from 2:1 to 5:1. In steps II and III the ratios vary from between 2:1 to 8:1 for solvents of relatively high solvent power such as methyl isobutyl ketone to from about 8:1 to 20:1 for solvents of relatively low solvent power such as methyl ethyl ketone. If the solvent power of a low solvency solvent is raised, as by the addition of toluene, the desired ratio may be reduced to below 8:1.

For washing the cakes amounts of solvent normally vary between  $\frac{1}{2}:1$  to 3:1 times its volume, and preferably about 2:1.

We claim as our invention:

1. A process for separating liquid non-aromatic hydrocarbons from liquid aromatic hydrocarbons in a mixture thereof having an initial boiling point of above about  $200^{\circ}$  C. and containing dissolved between about 5% and 25% by volume of normally solid wax, comprising treating said mixture with at least about an equal volume of a first polar solvent having a preferential solubility for aromatic hydrocarbons, cooling the resulting mixture to a temperature below about  $-50^{\circ}$  C. to produce a solid phase comprising at least a major portion of the non-aromatic hydrocarbons and a liquid phase comprising said first solvent and said aromatic hydrocarbons, separating said phases, treating said separated solid phase with a second polar solvent at a temperature higher than that in the first cooling stage but below about  $0^{\circ}$  C. to produce a second solid wax phase and a second liquid phase comprising said liquid non-aromatic hydrocarbons and said second polar solvent, and separating said second solid wax phase from said second liquid phase.

2. The process of claim 1, where in said second polar solvent is the same as said first polar solvent.

3. A process for separating low viscosity index oil from high viscosity index oil in a petroleum distillate having an initial boiling temperature above about  $200^{\circ}$  C. and containing dissolved between about 5 and 25% by volume of a normally solid wax, comprising treating said distillate with at least about an equal volume of a selective solvent for said low viscosity index components, cooling the resulting mixture to a temperature below about  $-50^{\circ}$  C. to produce a solid phase comprising at least a major portion of said high

viscosity index components and wax and a liquid phase comprising said selective solvent and said low viscosity index components, separating said phases, treating the separated solid phase with a polar solvent at a temperature higher than that employed in producing the first solid phase but below about 0° C. to produce a second solid phase and a second liquid phase comprising the high viscosity index components of said distillate, and separating said second solid phase from said high viscosity index components.

4. A process for separating liquid non-aromatic hydrocarbons from liquid aromatic hydrocarbons in a mixture thereof having an initial boiling temperature above about 200° C. comprising treating said mixture in the presence of between about 5 and 25% by volume of a normally solid wax dissolved therein, with at least about an equal volume of a ketone having a preferential solubility for aromatic hydrocarbons, cooling the resulting mixture to a temperature below about -50° C. to produce a solid phase comprising at least a major portion of the non-aromatic hydrocarbons and wax and a liquid phase comprising said ketone and said aromatic hydrocarbons, separating said phases, treating said separated solid phase with a solvent at a temperature higher than that used in obtaining the first solid phase but below about 0° C. to produce a second solid wax phase and a second liquid phase comprising said liquid non-aromatic hydrocarbons and said solvent, and separating said second solid wax phase from said second liquid phase.

5. A process for separating liquid non-aromatic hydrocarbons from liquid aromatic hydrocarbons in a mixture thereof having an initial boiling temperature of above about 200° C. and containing dissolved between about 5 and 25% by volume of a normally solid wax comprising treating said mixture with at least about an equal volume of a polar solvent having a preferential solubility for aromatic hydrocarbons and thereby forming a resulting mixture which upon cooling sufficiently yields a gelatinous mass which increases in viscosity as the temperature is lowered progressively until a critical low temperature is reached at which the viscosity of the resulting mixture decreases, cooling the resulting mixture to a temperature at least as low as said critical low temperature and producing a solid phase comprising said wax and at least a major portion of the non-aromatic hydrocarbons and a liquid phase comprising said solvent and said aromatic hydrocarbons, separating said phases, treating said separated solid phase with a second solvent at a temperature higher than that in the first cooling stage to produce a second solid wax phase and a second liquid phase comprising said liquid non-aromatic hydrocarbons and said second solvent, and separating said second solid wax phase from said second liquid phase.

6. A process for obtaining crystalline wax from a mixture of liquid non-aromatic hydrocarbons, substantially devoid of aromatic hydrocarbons, which mixture possesses an initial boiling temperature above about 200° C. and contains at least 5% by volume of a normally solid wax dissolved therein comprising treating said mixture with at least an equal volume of a solvent comprising a ketone and an aromatic hydrocarbon and thereby forming a resulting mixture which upon cooling sufficiently yields a gelatinous mass which increases in viscosity as the temperature is lowered progressively until a critical low temperature is reached at which the viscosity of the

resulting mixture decreases, cooling the resulting mixture to a temperature at least as low as said critical low temperature and producing a liquid phase and a solid phase, separating the two phases and treating said separated solid phase at a higher temperature with at least an equal volume of a ketone containing solvent to produce a solid phase essentially containing crystalline wax and a liquid phase essentially containing said solvent and amorphous wax dissolved therein and separating these latter two phases.

7. A process for separating a liquid hydrocarbon mixture having an initial boiling temperature above about 200° C. and containing aromatic hydrocarbons and non-aromatic hydrocarbons including amorphous wax, comprising treating said mixture in the presence of at least 5% by volume of a normally solid crystalline wax dissolved therein with at least about an equal volume of a first solvent which has a selective solubility for aromatic hydrocarbons and thereby forming a resulting mixture which upon cooling sufficiently yields a gelatinous mass which increases in viscosity as the temperature is lowered progressively until a critical low temperature is reached at which the viscosity of the resulting mixture decreases, cooling the resulting mixture to a temperature at least as low as said critical low temperature and producing a first liquid phase containing said first solvent and said aromatics and a first solid phase containing said non-aromatics and said waxes, separating said phases, treating said separated first solid phase at a substantially higher temperature with at least an equal volume of a second solvent to produce a second liquid phase containing said second solvent and said non-aromatic hydrocarbons and a second solid phase containing said waxes, separating said second phases, treating said separated second solid phase at a still higher temperature with at least an equal volume of a third solvent to produce a third liquid phase containing said third solvent and said amorphous wax and a third solid phase containing said normally solid crystalline wax, and separating said third phases.

8. The process of claim 7, wherein said first, said second and said third solvents are the same.

9. The process of claim 7, wherein said first, said second and said third solvents contain a ketone.

10. The process of claim 3 wherein said selective solvent and said polar solvent are the same.

11. A process for separating non-aromatic hydrocarbons from aromatic hydrocarbons in a liquid mixture thereof having an initial boiling temperature of above about 200° C. and containing dissolved therein at least about 5% by volume of a normally solid wax comprising treating said mixture with a solvent having a preferential solubility for aromatic hydrocarbons and thereby forming a resulting mixture which upon cooling sufficiently yields a gelatinous mass which increases in viscosity as the temperature is lowered progressively until a critical low temperature is reached at which the viscosity of the resulting mixture decreases, cooling the resulting mixture to a temperature at least as low as said critical low temperature and producing a solid phase comprising said wax and at least a major portion of the non-aromatic hydrocarbons and a liquid phase comprising said solvent and said aromatic hydrocarbons, separating said phases, treating said separated solid phase with a second solvent at a temperature higher than that in the first

9

cooling stage to produce a second solid wax phase and a second liquid phase comprising said liquid non-aromatic hydrocarbons and said second solvent, and separating said second solid wax phase from said second liquid phase.

12. A process for separating components of a liquid hydrocarbon mixture having an initial boiling temperature above about 200° C. and containing aromatic hydrocarbons and non-aromatic hydrocarbons including amorphous wax, comprising treating said mixture in the presence of at least 5% by volume of a normally solid crystalline wax dissolved therein with a first solvent having a preferential solubility for aromatic hydrocarbons and thereby forming a resulting mixture which upon cooling sufficiently yields a gelatinous mass which increases in viscosity as the temperature is lowered progressively until a critical low temperature is reached at which the viscosity of the resulting mixture decreases, cooling the resulting mixture to a temperature at least as low as said critical low temperature and producing a first liquid phase containing said first solvent and said aromatics and a first solid phase containing said non-aromatics and said waxes, separating said phases, treating said separated first solid phase at a substantially higher temperature with a second solvent to produce a second liquid phase containing said second solvent and said non-aromatic hydrocarbons and a second solid phase containing said waxes, separating said second phases, treating said separated second solid phase at a still higher temperature with

10

a third solvent to produce a third liquid phase containing said third solvent and said amorphous wax and a third solid phase containing said normally solid crystalline wax, and separating said third phases.

13. The process of claim 5, wherein said polar solvent comprises methyl isobutyl ketone.

14. The process of claim 5, wherein said polar solvent comprises methyl ethyl ketone.

10

HALL STEWART.  
AUGUST A. SCHAEERER.

## REFERENCES CITED

The following references are of record in the file of this patent:

## UNITED STATES PATENTS

| Number       | Name            | Date          |
|--------------|-----------------|---------------|
| 1,669,151    | Wagner          | May 8, 1928   |
| 20 1,951,780 | Voorhees        | Mar. 20, 1934 |
| 1,980,649    | Voorhees et al. | Nov. 13, 1934 |
| 2,108,629    | Van Wijk        | Feb. 15, 1938 |
| 2,161,569    | Gross           | June 6, 1939  |
| 2,164,013    | Jenkins         | June 27, 1939 |
| 25 2,180,763 | Nederbragt      | Nov. 21, 1939 |
| 2,193,767    | Manley et al.   | Mar. 12, 1940 |
| 2,198,576    | Govers          | Apr. 23, 1940 |
| 2,234,916    | Jones           | Mar. 11, 1941 |
| 2,246,982    | Nederbragt      | June 24, 1941 |

30

## FOREIGN PATENTS

| Number  | Country       | Date          |
|---------|---------------|---------------|
| 441,104 | Great Britain | Jan. 13, 1936 |